# EUROPEAN PATENT SPECIFICATION

(11) **EP 2 602 347 B1**
(45) Date of publication and mention of the grant of the patent: **20.02.2019**
(21) Application number: 11814324.7
(22) Date of filing: 05.08.2011
(51) Int. Cl.: C22C 38/00, C21D 8/12, H01F 1/16, C22C 38/60, C21D 1/38, C22C 38/04, C22C 38/34

(54) **GRAIN-ORIENTED MAGNETIC STEEL SHEET AND PROCESS FOR PRODUCING SAME**
KORNORIENTIERTES MAGNETISCHES STAHLBLECH UND HERSTELLUNGSVERFAHREN DAFÜR
TÔLE D'ACIER MAGNÉTIQUE À GRAINS ORIENTÉS ET SON PROCÉDÉ DE PRODUCTION

(30) Priority: 06.08.2010 JP 2010178136
(43) Date of publication of application: 12.06.2013
(73) Proprietor: JFE Steel Corporation, Tokyo 100-0011 (JP)
(72) Inventor: INOUE, Hirotaka, Tokyo 100-0011 (JP); YAMAGUCHI, Hiroi, Tokyo 100-0011 (JP); OKABE, Seiji, Tokyo 100-0011 (JP); OMURA, Takeshi, Tokyo 100-0011 (JP)
(74) Representative: Grünecker Patent- und Rechtsanwälte PartG mbB
(86) International application number: PCT/JP2011/004477
(87) International publication number: WO 2012/017693

(56) References cited:
- JP-A- 1 191 744
- JP-A- 3 260 020
- JP-A- 3 260 020
- JP-A- 3 287 725
- JP-A- 7 090 385
- JP-A- 10 183 313
- JP-A- 56 105 420
- JP-A- 56 105 424
- JP-A- 56 105 426
- JP-A- 57 188 811
- JP-A- 59 023 822
- JP-A- 59 023 822
- JP-A- 61 235 514
- JP-A- 2003 034 822
- JP-A- 2004 124 226
- US-A- 4 363 677
- US-A- 4 613 842
- US-A- 6 083 326

## Description

### TECHNICAL FIELD

The present invention relates to a grain oriented electrical steel sheet advantageously utilized for an iron core of a transformer and the like and a method for manufacturing a grain oriented electrical steel sheet advantageously utilized for an iron core of a transformer and the like.

### BACKGROUND ART

A grain oriented electrical steel sheet is mainly utilized as an iron core of a transformer and required to exhibit superior magnetization characteristics, e.g. low iron loss in particular.
In this regard, it is important to highly accumulate secondary recrystallized grains of a steel sheet in (110)[001] orientation, i.e. what is called "Goss orientation", and reduce impurities in a product steel sheet. However, there are restrictions on controlling crystal grain orientations and reducing impurities in view of production cost. Accordingly, there has been developed a technique of introducing non-uniformity into a surface of a steel sheet by physical means to subdivide width of a magnetic domain to reduce iron loss, i.e. magnetic domain refinement technique.

For example, Patent Literature 1 proposes a technique of irradiating a steel sheet as a finished product with laser to introduce high-dislocation density regions into a surface layer of the steel sheet, thereby narrowing magnetic domain widths and reducing iron loss of the steel sheet. Patent Literature 2 suggests a technology for controlling magnetic domain widths by irradiating electron beam. PTL 3 and PTL 4 disclose laser irradiation of electromagnetic steel sheets.

### CITATION LIST

### Patent Literature

PTL 1: JP-B 57-002252
PTL 2: JP-B 06-072266
PTL 3: US 4,363,677
PTL 4: US 4,613,842

### SUMMARY OF THE INVENTION

### Technical Problems

However, in the case where a grain oriented electrical steel sheet with reduced iron loss obtained by conducting above-mentioned magnetic domain refinement technique including irradiation of laser or electron beam is adapted to an actual transformer, there was a problem in which the iron loss property of the actual transformer was not improved even if the iron loss of the material (steel sheet) was thus reduced. That is, a building factor (BF) became poor, in such case.

Therefore, an object of the present invention is to provide a grain oriented electrical steel sheet capable of reducing iron loss, even in the case where the grain oriented electrical steel sheet is stacked and adapted to an iron core of a transformer or the like, by conducting magnetic domain refinement treatment.

### Solution to the Problems

In order to reduce iron loss of a grain oriented electrical steel sheet utilized as an iron core of a transformer, that is, in order to reduce an iron loss of the transformer itself, the iron loss in a direction other than the rolling direction as well as the iron loss in a rolling direction of the steel sheet needs to be reduced.

Regarding the magnetized status in the transformer during excitation, a phenomenon called as magnetization rotation is known to occur. In magnetization rotation, the magnetization direction is oriented to a direction other than the rolling direction when magnetic excitation is provided in a direction parallel to the rolling direction. In the case where a transformer with a three-phase and three-leg iron core is excited at magnetic flux density of 1.7 T in a direction parallel to the rolling direction, for example, the inventors of the present invention have found that magnetic flux of 0.1 T to 1.0 T is at least locally oriented along the direction orthogonal to the rolling direction. When the magnetization direction is oriented to a direction other than the rolling direction in a grain oriented electrical steel sheet, the magnetization direction is eventually directed to the direction having low magnetic permeability and whereby the iron loss is increased. Such increase in iron loss caused by magnetization rotation is a cause for generating transformer iron loss larger than iron loss of the material itself (iron loss in the rolling direction).

An index for expressing the deterioration in magnetic property is called as BF (Building Factor), the value obtained from dividing the value of iron loss at a transformer by a value of iron loss at the material under the same magnetization condition. It is important to reduce iron loss in a direction other than the rolling direction, especially in a direction orthogonal to the rolling direction for reducing the value of BF.

Therefore, inventors of the present invention have introduced strain-imparted areas having appropriate sizes thermally in a dotted line pattern with appropriate intervals between the adjacent strain-imparted areas. The inventors eventually have found that both iron loss values in the rolling direction and the direction orthogonal to the rolling direction are reduced and a grain oriented electrical steel sheet exhibiting smaller value of transformer iron loss is eventually obtained.

Here, the principle for explaining the reduction in iron loss caused by strain imparting is set forth below. That is, when strain is imparted into a steel sheet, tension is introduced in a direction of the dotted-line so as to generate a closure domain originated from the strain. On one hand, the generation of the closure domain increases magnetostatic energy and on the other hand, the 180° magnetic domain is subdivided for reducing the increased magnetostatic energy. Accordingly, the iron loss in the rolling direction is reduced. In the case where the larger amount of strain is imparted and the more closure domain is generated, the 180° magnetic domains will be subdivided further and the iron loss in the rolling direction will be reduced further. The increased tension in a direction of the dotted line causes a larger value of magnetic permeability in a direction orthogonal to the rolling direction by inverse magnetostriction effect and the iron loss in the direction orthogonal to the rolling direction is eventually reduced. Regarding the iron loss in the rolling direction, eddy current loss is reduced by narrowing the widths of magnetic domains by increasing the amount of strain to a level over or equal to an appropriate level, while a hysteresis loss increases and the iron loss in the rolling direction gets larger totally. In the case where density of strain-imparted areas in a steel sheet is high, the hysteresis loss in the rolling direction and the direction orthogonal to the rolling direction is increased, since the strain-imparted areas inhibit magnetic flow.

Based on the above, when appropriate amount of strain is imparted into the steel sheet at an appropriate density of strain-imparted areas, iron losses in both rolling direction and the direction orthogonal to the rolling direction can be reduced so that a grain oriented electrical steel sheet exhibiting lower transformer iron loss can be manufactured.

Next, to determine the appropriate condition for strain-imparting, an electron beam is irradiated according to variety of irradiation conditions and the size of strain-imparted regions and the intervals between the adjacent strain-imparted regions in each steel sheet are investigated. The measurement methods for the size of strain-imparted regions and the intervals will be described later. The changes in values of W_{17/50} in the rolling direction and the values of W_{2/50} in the direction orthogonal to the rolling direction before or after the irradiation were studied. The excitation level for the direction orthogonal to the rolling direction is determined by using the iron loss value for 0.2 T as an index. Such value corresponds to an average value for a component of magnetic flux density in the direction orthogonal to the rolling direction, in a transformer for which the inventors conducted the research.

In an experiment, an electron beam having an acceleration voltage of 40 kV and beam current value of 2.5 mA was irradiated in a direction orthogonal to the rolling direction continuously or in a dotted line pattern having interval of 7 mm between irradiated lines, according to the condition shown in Table 1. The continuous irradiation was conducted at a beam scanning rate of 4 m/s, while the dotted line irradiation was conducted at a beam scanning rate of 50 m/s with 100 µs intermissions between predetermined time intervals which determine lengths of the space between irradiated dots. Samples subjected to the experiment were grain oriented electrical steel sheets having a thickness of 0.23 mm and having B₈ value before irradiation of approximately 1.93 T.

Definitions and measurement methods for the above-mentioned size of strain-imparted areas and the intervals between the adjacent strain-imparted areas are set forth below.

### [Size of Strain-Imparted Areas]

A surface coating of a steel sheet after subjected to final annealing was removed by acid or alkali, and then the hardness measurement was conducted by using nanoindenter for the strain-imparted areas. The hardness at the position at least 1 mm away from strain-imparted line was used as a standard and the areas of hardness that is higher than the hardness at the position by 10 % or more were defined as strain-imparted areas (i.e. strain-imparted areas distributed in a dotted line).

The maximum length in the direction orthogonal to the rolling direction within the strain-imparted area was defined as the size of strain-imparted area. In the continuous irradiation condition or in the condition where the strain-imparted areas corresponding to the neighboring dotted lines overlap each other, the maximum length in the rolling direction was defined as the size of strain-imparted area. The size of strain-imparted area was measured based on the above definitions. Specifically, the size of strain-imparted area was determined, for example, as the average value calculated based on each ten strain-imparted points, in the center portion of sample steel sheet, selected from three different dotted lines per one sheet.

### [Intervals between Adjacent Strain-Imparted Areas]

Between the above-defined strain-imparted areas, the minimum length free from the both effects of the adjacent strain-imparted areas was defined as the interval between the adjacent strain-imparted areas. In the continuous irradiation condition or in the condition where the strain-imparted areas corresponding to the neighboring dotted lines overlap each other, the interval between the adjacent strain-imparted areas was defined as 0 mm. On the basis of the above definitions, the interval between the adjacent areas was measured. The interval between the adjacent areas was determined, for example, as the average value calculated based on each ten strain-imparted points, in the center portion of sample steel sheet, selected from three different dotted lines per one sheet.

Table 1 shows the result of the study for the size of strain-imparted area and interval between the adjacent strain-imparted areas in each steel sheet in various irradiation conditions and in various intervals between irradiated dots in the direction orthogonal to the rolling direction. Figs. 1 and 2 show the change in values of W_{17/50} and W_{2/50} in the rolling direction as a function of the interval between the adjacent strain-imparted areas.

### Table 1

**Table 1**

| Condition | Irradiation | Irradiation interval in direction orthogonal to rolling direction (mm) | Beam diameter (mm) | Size of strain-imparted area (mm) | Dot interval between adjacent strain-imparted areas (mm) |
|---|---|---|---|---|---|
| 1 | Continuous | - | 0.2 | 0.27 | No interval |
| 2 | Dotted line | 1.2 | 0.2 | 0.28 | 0.78 |
| 3 | Dotted line | 0.9 | 0.2 | 0.28 | 0.59 |
| 4 | Dotted line | 0.7 | 0.2 | 0.29 | 0.36 |
| 5 | Dotted line | 0.5 | 0.2 | 0.29 | 0.15 |
| 6 | Dotted line | 0.4 | 0.2 | 0.29 | 0.08 |
| 7 | Dotted line | 0.3 | 0.2 | 0.32 | No interval |
| 8 | Continuous | - | 0.1 | 0.16 | No interval |
| 9 | Dotted line | 1.2 | 0.1 | 0.17 | 1.02 |
| 10 | Dotted line | 0.9 | 0.1 | 0.17 | 0.7 |
| 11 | Dotted line | 0.7 | 0.1 | 0.18 | 0.48 |
| 12 | Dotted line | 0.5 | 0.1 | 0.18 | 0.25 |
| 13 | Dotted line | 0.3 | 0.1 | 0.19 | 0.05 |
| 14 | Dotted line | 0.2 | 0.1 | 0.21 | No interval |

As Shown in Fig. 1, in the case where the interval between the adjacent strain-imparted areas was 0.60 mm or less, the value of W_{17/50} in the rolling direction corresponded to smaller value. The value of iron loss got smaller since the narrower intervals between the adjacent strain-imparted areas resulted in the larger amount of stain imparted which caused magnetic domain refining effect.

On the other hand, as shown in Fig. 2, the value of iron loss W_{2/50} in the direction orthogonal to the rolling direction decreased by 10 % or more from the values for continuous irradiation, when the dotted line irradiation was conducted under a condition in which the interval between the adjacent strain-imparted areas was at least 0.10 mm. This phenomenon occurred presumably because the increase in hysteresis loss in the direction orthogonal to the rolling direction was suppressed by minimizing the dimension of strain-imparted areas.

Next, the inventors of the present invention studied effects of the size of the strain-imparted areas. An electron beam at an acceleration voltage of 40 kV was irradiated in a dotted-line in a direction orthogonal to the rolling direction of the steel sheet with spacing of 7 mm in the rolling direction. The irradiation was conducted under a condition in which the beam diameter and the current density were adjusted so that interval between the adjacent strain-imparted areas ranged from 0.2 mm or more to 0.3 mm or less and the respective strain-imparted areas had different sizes. Fig. 3 shows the relation between the size of stain-imparted area and the value of iron loss. In the case where the size of stain-imparted area is between 0.1 mm or more and 0.5 mm or less, the value for W_{17/50} in the rolling direction got smaller. This phenomenon occurred presumably because the larger sizes of strain-imparted areas increased the amount of stain imparted to exert magnetic domain refining effect for reducing the iron loss. Once the stain larger than a certain amount was imparted, the hysteresis loss in the rolling direction got larger and iron loss accompanied it. As shown in Fig. 4, the value of iron loss W_{2/50} in the direction orthogonal to the rolling direction got smaller when the size of stain-imparted area is 0.1 mm or more. This phenomenon occurred presumably because closure magnetic domain capable of decreasing iron loss in the direction orthogonal to the rolling direction could not develop sufficiently when the size of strain-imparted area was less than 0.1 mm.

Based on such experimental results, the inventors of the present invention found that both values of iron losses in the rolling direction and the direction orthogonal to the rolling direction decreased when strain was imparted in a dotted-line for obtaining the appropriate size of strain-imparted areas and the interval between the adjacent strain-imparted areas. Accordingly, the inventors of the present invention have obtained the grain oriented electrical steel sheet having low transformer iron loss.

Specifically, primary features of the present invention are set out in the appended claims.

### Advantageous Effect of the Invention

It is possible to reduce iron losses in both the rolling direction and the direction orthogonal to the rolling direction by imparting strain in a dotted-line arrangement under restrictions according to the present invention. Thus, it is possible to further reduce iron loss in a transformer provided with stacked grain oriented electrical sheets obtained as above.

### BRIEF DESCRIPTION OF DRAWINGS

The present invention will be further described below with reference to the accompanying drawings, wherein:
FIG. 1 is a graph showing relationships between the interval between the adjacent strain-imparted areas and iron loss;
FIG. 2 is a graph showing relationships between the interval between the adjacent strain-imparted areas and iron loss;
FIG. 3 is a graph showing relationships between the size of strain-imparted area and iron loss;
FIG. 4 is a graph showing relationships between the size of strain-imparted area and iron loss; and
FIG. 5 is a diagram illustrating a shape of the transformer iron core.

### DESCRIPTION OF EMBODIMENTS

As mentioned above, it is necessary to reduce iron losses in both the rolling direction and the direction orthogonal to the rolling direction for reducing iron loss in a transformer. On one hand, it is important to form thermal strain-imparted areas under a condition capable of satisfying the size of strain-imparted area between 0.10 mm or more and 0.50 mm or less and the interval between the adjacent strain-imparted areas of 0.60 mm or less, in order to reduce iron loss in the rolling direction. On the other hand, it is important to form thermal strain-imparted areas under a condition capable of satisfying the size of strain-imparted area of 0.10 mm or more and the interval between the adjacent strain-imparted areas of 0.10 mm or more, in order to reduce iron loss in the direction orthogonal to the rolling direction.

Further, the line interval in the rolling direction between the strains imparted in dotted-line arrangement is set between 2 mm or more and 10 mm or less. In the case where the line interval is less than 2 mm, the amount of strains imparted into the steel sheet is too much and hysteresis loss increases significantly in the rolling direction. On the other hand, in the case where the line interval exceeds 10 mm, the magnetic domain refining effect is reduced and whereby iron loss in both rolling direction and the direction orthogonal to the rolling direction increase.

Further, strains imparted in a dotted-line arrangement in a direction that crosses the rolling direction of a steel sheet is disposed for having an angle within 30° between the dotted line and the direction orthogonal to the rolling direction. In the case where the tilting angle against the direction orthogonal to the rolling direction exceeds such range, the decrease of iron loss in the rolling direction is suppressed even though the iron loss in the direction orthogonal to the rolling direction decreases, and eventually the decrease in iron loss for a transformer is suppressed. More preferably, the strains are imparted along the direction orthogonal to the rolling direction.

By satisfying the above mentioned condition, an appropriate amount of strain is imparted into a steel sheet for generating closure magnetic domains so that iron loss in both the rolling direction and the direction orthogonal to the rolling direction decreased sufficiently, and eventually a grain oriented electrical steel sheet, optimal for the reduction in iron loss in a transformer as intended in the present invention, is obtained. Outside of such appropriate range, in the case where the amount of strain imparted is insufficient, the effect of reducing iron loss is suppressed, and in the case where the amount of stain imparted is too much or the stain-imparted area is too large, the hysteresis loss significantly increases and the effect of reducing iron loss is suppressed.

Next, the manufacturing method for imparting thermal strains under the above mentioned condition will be set forth below.

First, as an introduction method for dotted-line strains, it is suitable to utilize an electron beam irradiation or a continuous laser irradiation capable of introducing huge energy by a focused beam diameter. As other magnetic domain refining method, means of plasma-jet irradiation is known and it is difficult to adapt such means within the condition of the present invention.

### (i) Introduction of thermal strains by means of electron beam irradiation

Irradiation condition was studied for introducing the above defined thermal strains by conducting experiments for electron beams of different intervals between dotted-lines and irradiation energy amount E. The irradiation energy amount E is defined by the formula below. $E \left(mJ/mm\right) = \left[Acceleration voltage of electron beam \left(kV\right)\times Beam current value \left(mA\right)\times Irradiation period per one dot \left(μs\right)/1,000\right] / Beam diameter \left(mm\right)$

The beam diameter is determined by a known slit method using a half width of energy profile.

As a result of the above study, it has been revealed that the above identified condition for introducing strains is satisfied in the case where the line interval in the rolling direction for the electron beam irradiation is between from 2 mm to 10 mm; an irradiated dot interval in the dotted-line arrangement is from 0.2 mm or more to 1. 0 mm or less; and an irradiation energy amount E per unit beam diameter is 30 mJ/mm or more and 180 mJ/mm or less.

### (ii) Introduction of thermal strains by means of continuous laser irradiation

Irradiation condition was studied for continuous laser irradiation in the range satisfying the above condition in the same manner. The irradiation energy amount E is defined by the formula below. $E \left(mJ/mm\right) = \left[Average laser power \left(W\right)\times Irradiation period per one dot \left(μs\right)/1,000\right] / Beam diameter \left(mm\right)$

As a result of the above study, it has been revealed that the above identified condition for introducing strains is satisfied in the case where the line interval in the rolling direction for the irradiation of laser is between 2 mm and 10 mm; an irradiated dot interval in the dotted-line arrangement is from 0.2 mm or more to 1. 0 mm or less; and an irradiation energy amount E per unit beam diameter is 40 mJ/mm or more and 200 mJ/mm or less.

The laser oscillation can be switched off or switched to low power, when a laser beam moves between irradiation dots. The beam diameter can be set uniquely based on collimator and a focal length of a lens in an optical system.

The method for introducing strains in the dotted-line arrangement is realized by repeating a process in which an electron beam or a laser beam rapidly scans across a steel sheet while the scan is stopped at every dot for a given time period, the irradiation continues at the dot, and then the scan restarts. Such process can be realized by means of an electron beam irradiation in which a diffraction voltage of the electron beam is varied by using an amplifier having large capacity.

When a steel sheet is subjected to strain introduction in the dotted-line arrangement by means of an electron beam or a continuous laser beam, the resultant steel sheet have irradiation traces and an electrical insulation property of the steel sheet may be compromised. In such case, recoating of the insulating coating is conducted and the coating thus applied is baked at a temperature range in which the introduced strain is not compensated.

Next, a manufacturing condition for a grain oriented electrical steel sheet other than the above-identified condition will be concretely explained. It is preferable to have magnetic flux density B₈ of 1.90 T or more, which can be an indicator of degrees of accumulation, since the higher degrees of accumulation in <100> direction among crystal grains leads to the higher iron loss reduction effect caused by magnetic domain refining.

In the chemical composition of a slab for the grain oriented electrical steel sheet according to the present invention may be any chemical composition as long as the composition can cause secondary recrystallization. Further, in a case of using an inhibitor, for example, in a case of using AlN inhibitor, an appropriate amount of Al and N may be contained while in a case of using MnS and/or MnSe inhibitor, an appropriate amount of Mn and Se and/or S may be contained. It is needless to say that both of the inhibitors may also be used in combination. Preferred contents of Al, N, S, and Se in this case are as follows: Al: 0.01 mass% to 0.065 mass%; N: 0.005 mass% to 0.012 mass%; S: 0.005 mass% to 0.03 mass%; and Se: 0.005 mass% to 0.03 mass%.

Further, the present invention can also be applied to a grain oriented electrical steel sheet in which the contents of Al, N, S, and Se are limited and no inhibitor is used. In this case, the amounts of Al, N, S, and Se each may preferably be suppressed as follows: Al: 100 mass ppm or below; N: 50 mass ppm or below; S: 50 mass ppm or below; and Se: 50 mass ppm or below.

Specific examples of basic components and other components to be optionally added to a steel slab for use in manufacturing the grain oriented electrical steel sheet of the present invention are as follows.

### C: 0.08 mass% or less

Carbon is added to improve texture of a hot rolled steel sheet. Carbon content in steel is preferably 0.08 mass% or less because carbon content exceeding 0.08 mass% increases burden of reducing carbon content during the manufacturing process to 50 mass ppm or less at which magnetic aging is reliably prevented. The lower limit of carbon content in steel need not be particularly set because secondary recrystallization is possible in a material not containing carbon.

### Si: 2.0 mass% to 8.0 mass%

Silicon is an element which effectively increases electrical resistance of steel to improve iron loss properties thereof. Silicon content in steel equal to or higher than 2.0 mass% ensures a particularly good effect of reducing iron loss. On the other hand, Si content in steel equal to or lower than 8.0 mass% ensures particularly good formability and magnetic flux density of a resulting steel sheet. Accordingly, Si content in steel is preferably in the range of 2.0 mass% to 8.0 mass%.

### Mn: 0.005 mass% to 1.0 mass%

Manganese is an element which advantageously achieves good hot-workability of a steel sheet. Manganese content in a steel sheet less than 0.005 mass% cannot cause the good effect of Mn addition sufficiently. Manganese content in a steel sheet equal to or lower than 1.0 mass% ensures particularly good magnetic flux density of a product steel sheet. Accordingly, Mn content in a steel sheet is preferably in the range of 0.005 mass% to 1.0 mass%.

Further, the steel slab for the grain oriented electrical steel sheet of the present invention may contain, for example, following elements as magnetic properties improving components in addition to the basic components described above.

### At least one element selected from Ni: 0.03 mass% to 1.50 mass%, Sn: 0.01 mass% to 1.50 mass%, Sb: 0.005 mass% to 1.50 mass%, Cu: 0.03 mass% to 3.0 mass%, P: 0.03 mass% to 0.50 mass%, Mo: 0.005 mass% to 0.10 mass%, and Cr: 0.03 mass% to 1.50 mass%

Nickel is a useful element in terms of further improving texture of a hot rolled steel sheet and thus magnetic properties of a resulting steel sheet. However, Nickel content in steel less than 0.03 mass% cannot cause this magnetic properties-improving effect by Ni sufficiently, while Nickel content in steel equal to or lower than 1.5 mass% ensures stability in secondary recrystallization to improve magnetic properties of a resulting steel sheet. Accordingly, Ni content in steel is preferably in the range of 0.03 mass% to 1.5 mass%.

Sn, Sb, Cu, P, Cr, and Mo each are a useful element in terms of improving magnetic properties of the grain oriented electrical steel sheet of the present invention. However, sufficient improvement in magnetic properties cannot be obtained when contents of these elements are less than the respective lower limits specified above. On the other hand, contents of these elements equal to or lower than the respective upper limits described above ensure the optimum growth of secondary recrystallized grains. Accordingly, it is preferred that the steel slab for grain oriented electrical steel sheet of the present invention contains at least one of Sn, Sb, Cu, P, Cr, and Mo within the respective ranges thereof specified above.

The balance other than the aforementioned components of the grain oriented electrical steel sheet of the present invention is Fe and incidental impurities incidentally mixed thereinto during the manufacturing process.

Next, the slab having the aforementioned chemical compositions is heated and then subjected to hot rolling, according to a conventional method. Alternatively, the casted slab may be immediately hot rolled without being heated. In a case of a thin cast slab/strip, the slab/strip may be either hot rolled or directly fed to the next process skipping hot rolling.

A hot rolled steel sheet (or the thin cast slab/strip which skipped hot rolling) is then subjected to hot-band annealing according to necessity. The main purpose of the hot-band annealing is to eliminate the band texture resulting from the hot rolling so as to have the primary recrystallized texture formed of uniformly-sized grains, so that the Goss texture is allowed to further develop in the secondary recrystallization annealing, to thereby improve the magnetic property. At this time, in order to allow the Goss texture to highly develop in the product steel sheet, the hot-band annealing temperature is preferably defined to fall within a range of 800 °C to 1,100 °C. At a hot-band annealing temperature lower than 800 °C, the band texture resulting from the hot rolling is retained, which makes it difficult to have the primary recrystallization texture formed of uniformly-sized grain, and thus a desired improvement in secondary recrystallization cannot be obtained. On the other hand, at a hot-band annealing temperature higher than 1,100 °C, the grain size is excessively coarsened after the hot-band annealing, which makes it extremely difficult to obtain a primary recrystallized texture formed of uniformly-sized grain.

After the hot-band annealing, the steel sheet is subjected to cold rolling at least once or at least twice, with intermediate annealing therebetween before being subjected to decarburizing annealing (which also serves as recrystallization annealing), which is then applied with an annealing separator. The steel sheet applied with an annealing separator is then subjected to final annealing for the purpose of secondary recrystallization and forming a forsterite film (film mainly composed of Mg₂SiO₄).

To form forsterite, an annealing separator mainly composed of MgO may preferably be used. Here, a separator mainly composed of MgO may also contain, in addition to MgO, a known annealing separator component or a property improvement component, without inhibiting the formation of a forsterite film intended by the present invention.

After the final annealing, it is effective to level the shape of the steel sheet through flattening annealing. Meanwhile, according to the present invention, the steel sheet surface is applied with a insulating coating before or after the flattening annealing. Here, the insulating coating refers to a coating capable of imparting tension to a steel sheet for the purpose of reducing iron loss (referred to as tension-imparting coating, hereinafter). The tension-imparting coating can be implemented by, for example, an inorganic coating containing silica or a ceramic coating applied by means of physical deposition, chemical deposition, and the like.

In the present invention, magnetic refinement is implemented by irradiating the surface of a grain oriented electrical steel sheet with an electron beam or a continuous laser beam under the above-described condition, after the final annealing or after the tension-imparting coating.

Processes or conditions other than the above described processes or manufacturing condition, the conventionally known manufacturing method for grain oriented electrical steel sheets including magnetic refinement processing using an electron beam or a continuous laser beam can be adapted in the present invention.

### Examples

A cold rolled sheet including Si at 3 mass% and having final sheet thickness of 0.23 mm was subjected to decarburizing and annealing for primary recrystallization; annealing separator mainly composed of MgO was applied to the steel sheet; and the steel sheet was subjected to final annealing including secondary recrystallization process and purification process, whereby a grain oriented electrical steel sheet having a forsterite film is obtained. Then, the steel sheet was applied with an insulating coating containing colloidal silica by 60 mass% and aluminum phosphate and the steel sheet was baked at 800 °C. Then, the steel sheet was irradiated with an electron beam or laser beam in a direction orthogonal to the rolling direction such that introducing strains into the steel sheet in dotted-line arrangement or continuous line arrangement. In dotted line irradiation, the interval between the direction orthogonal to the rolling direction was varied by controlling the stop time period in beam scanning. Accordingly, a steel material having magnetic flux density B₈ in the range of 1.90 T to 1.94 T was obtained.

The steel material thus obtained was sheared into specimens, having bevel edges, with shape and dimension as shown in FIG. 5 and stacked alternately in 70 layers such that assembling a three-phase and three-leg type transformer iron core of 500 mm square. The transformer was excited at magnetic flux density of 1.7 T and excitation frequency of 50 Hz and non-load loss (i.e. transformer iron loss) was measured by a power meter.
The measured values for transformer iron loss are shown in Tables 2 and 3 together with parameters including irradiation condition, size of strain-imparted area, and interval between the adjacent strain-imparted areas.

### Table 2

**Table 2**

| Cndition | Irradiation | Irradiation condition | | | | | | | Strain-imparted area | | B₈(T) | Iron loss of transformer W_{17/50} (W/kg) | Remark |
|---|---|---|---|---|---|---|---|---|---|---|---|---|---|
| | | Line Interval (mm) | Dot interval (mm) | Acceleration voltage (kV) | Beam current value (mA) | irradiation period per one dot (µs) | Beam diameter (mm) | E (mJ/mm) | Size of strain-imparted area (mm) | Interval between adjacent strain- | | | |
| 1 | Erectron beam/Dotted line | 7 | 0.4 | 150 | 0.5 | 40 | 0.2 | 15.0 | 0.08 | 0.24 | 1.93 | 0.92 | Comparative Example |
| 2 | Erectron beam/Dotted line | 3 | 0.1 | 150 | 0.8 | 40 | 0.2 | 24.0 | 0.12 | 0 | 1.92 | 0.9 | Comparative Example |
| 3 | Erectron beam/Dotted line | 3 | 1.0 | 150 | 0.5 | 60 | 0.2 | 22.5 | 0.12 | 0.8 | 1.94 | 0.92 | Comparative Example |
| 4 | Erectron beam/Dotted line | 3 | 0.5 | 150 | 3 | 100 | 0.2 | 225.0 | 0.55 | 0 | 1.92 | 0.9 | Comparative Example |
| 5 | Erectron beam/Dotted line | 5 | 0.8 | 120 | 2.5 | 80 | 0.15 | 160.0 | 0.47 | 0.27 | 1.92 | 0.86 | Inventive Example |
| 6 | Erectron beam/Dotted line | 5 | 0.5 | 40 | 1.5 | 100 | 0.15 | 40.0 | 0.19 | 0.3 | 1.94 | 0.85 | Inventive Example |
| 7 | Erectron beam/Dotted line | 3 | 0.9 | 40 | 2.5 | 100 | 0.2 | 50.0 | 0.31 | 0.59 | 1.93 | 0.84 | Inventive Example |
| 8 | Erectron beam/Dotted line | 3 | 0.4 | 80 | 2.5 | 40 | 0.15 | 53.3 | 0.23 | 0.12 | 1.92 | 0.86 | Inventive Example |
| 9 | Erectron beam/Dotted line | 1.5 | 0.9 | 40 | 2.5 | 100 | 0.2 | 50.0 | 0.29 | 0.58 | 1.90 | 0.94 | Comparative Example |
| 10 | Erectron beam/Dotted line | 11 | 0.9 | 40 | 2.5 | 100 | 0.2 | 50.0 | 0.33 | 0.55 | 1.94 | 0.90 | Comparative Example |
| 11 | Erectron beam/Dotted line | 5 | 1.2 | 40 | 1.5 | 100 | 0.15 | 40.0 | 0.45 | 0.72 | 1.94 | 0.92 | Comparative Example |
| 12 | Electron beam/ Cotinuous line | 5 | - | 150 | 0.5 | Scanning rate 5 m/s | 0.2 | - | 0.14 | - | 1.92 | 0.91 | Comparative Example |
| 13 | No irradiation | - | - | - | - | - | - | - | - | - | 1.94 | 1.05 | Comparative Example |

### Table 3

**Table 3**

| Condition | Irradiation | Irradiation condition | | | | | | Strain-imparted area | | B₈(T) | Iron loss of transformer W_{17/50} (W/kg) | Remark |
|---|---|---|---|---|---|---|---|---|---|---|---|---|
| | | Line Interval (mm) | Dot interval (mm) | Average laser power (W) | Irradiation period per one dot (µs) | Beam diameter (mm) | E (mJ/mm) | Size of strain-imparted area (mm) | Interval between adjacent strain-imparted areas (mm) | | | |
| 1 | Continuous laser/Dotted line | 7 | 0.3 | 180 | 10 | 0.1 | 18.0 | 0.08 | 0.22 | 1.93 | 0.91 | Comparative Example |
| 2 | Continuous laser/Dotted line | 3 | 0.1 | 180 | 10 | 0.1 | 18.0 | 0.09 | 0 | 1.93 | 0.91 | Comparative Example |
| 3 | Continuous laser/Dotted line | 3 | 1.2 | 250 | 30 | 0.1 | 75.0 | 0.24 | 1.02 | 1.94 | 0.90 | Comparative Example |
| 4 | Continuous laser/Dotted line | 3 | 0.6 | 250 | 140 | 0.15 | 233.3 | 0.53 | 0.05 | 1.92 | 0.90 | Comparative Example |
| 5 | Continuous laser/Dotted line | 5 | 1.0 | 200 | 40 | 0.15 | 53.3 | 0.22 | 0.75 | 1.93 | 0.89 | Comparative Example |
| 6 | Continuous laser/Dotted line | 5 | 0.4 | 250 | 20 | 0.1 | 50.0 | 0.18 | 0.15 | 1.93 | 0.85 | Inventive Example |
| 7 | Continuous laser/Dotted line | 3 | 0.8 | 200 | 50 | 0.15 | 66.7 | 0.23 | 0.55 | 1.93 | 0.85 | Inventive Example |
| 8 | Continuous laser/Dotted line | 3 | 0.6 | 250 | 100 | 0.15 | 166.7 | 0.41 | 0.13 | 1.92 | 0.84 | Inventive Example |
| 9 | Continuous laser/Dotted line | 1.5 | 0.4 | 250 | 20 | 0.1 | 50.0 | 0.17 | 0.19 | 1.90 | 0.93 | Comparative Example |
| 10 | Continuous laser/Dotted line | 11 | 0.4 | 250 | 20 | 0.1 | 50.0 | 0.20 | 0.16 | 1.93 | 0.91 | Comparative Example |
| 11 | Continuous laser/ Continuous line | 5 | - | 250 | Scanning rate 12 m/s | 0.15 | - | - | - | 1.93 | 0.90 | Comparative Example |
| 12 | No irradiation | - | - | - | - | - | - | - | - | 1.94 | 1.05 | Comparative Example |

As shown in Tables 2 and 3, in every inventive examples where thermal strains were appropriately introduced by means of an electron beam or continuous laser beam at appropriate size of strain-imparted area and appropriate interval between the adjacent strain-imparted areas, the transformer iron loss decreased by 5 % than comparative examples.

## Claims

1. A grain oriented electrical steel sheet having thermal strain introduced thereinto in a dotted-line arrangement in which strain-imparted areas have been lined in a direction that crosses the rolling direction of the steel sheet, wherein the strain-imparted areas introduced in the dotted-line arrangement have a size from 0.10 mm or more to 0.50 mm or less and an interval between the adjacent strain-imparted areas is from 0.10 mm or more to 0.60 mm or less, and a line interval between the dotted-lines in the rolling direction is from 2 mm to 10 mm.

2. A method for manufacturing a grain oriented electrical steel sheet, comprising:
introducing thermal strain into a grain oriented electrical steel sheet in a dotted-line arrangement in which strain-imparted areas have been lined in a direction that crosses the rolling direction of the steel sheet by irradiating an electron beam, wherein a line interval between the electron beam irradiation in the rolling direction is from 2 mm to 10 mm, an irradiated dot interval in the dotted-line arrangement is from 0.2 mm or more to 1. 0 mm or less, the strain-imparted areas introduced in the dotted-line arrangement have a size from 0.10 mm or more to 0.50 mm or less and an interval between the adjacent strain-imparted areas is from 0.10 mm or more to 0.60 mm or less, and an irradiation energy amount E per unit beam diameter defined by the following formula (1) is 30 mJ/mm or more and 180 mJ/mm or less, wherein: $E = \left[Acceleration voltage of electron beam \left(kV\right)\times Beam current value \left(mA\right)\times Irradiation period per one dot \left(μs\right)/1000\right] / Beam diameter \left(mm\right)$

3. A method for manufacturing a grain oriented electrical steel sheet, comprising:
introducing a thermal strain into a grain oriented electrical steel sheet in a dotted-line arrangement in which strain-imparted areas have been lined in a direction that crosses the rolling direction of the steel sheet by continuously irradiating a laser beam, wherein a line interval between the continuous laser irradiation in the rolling direction is from 2 mm to 10 mm, an irradiated dot interval in the dotted-line arrangement is from 0.2 mm or more to 1. 0 mm or less, the strain-imparted areas introduced in the dotted-line arrangement have a size from 0.10 mm or more to 0.50 mm or less and an interval between the adjacent strain-imparted areas is from 0.10 mm or more to 0.60 mm or less, and an irradiation energy amount E per unit beam diameter defined by the following formula (2) is 40 mJ/mm or more and 200 mJ/mm or less, wherein: $E = \left[Average laser power \left(W\right)\times Irradiation period per one dot \left(μs\right)/1000\right] / Beam diameter \left(mm\right)$

## Patentansprüche

1. Ein kornorientiertes Elektrostahlblech mit darin eingebrachter thermischer Spannung in einer gepunkteten Linien-Anordnung, in der die belasteten Bereiche in einer die Walzrichtung des Stahlblechs kreuzenden Richtung eingefasst wurden, wobei die belasteten Bereiche in die gepunktete Linien-Anordnung eingebracht wurden, die eine Größe von 0,10 mm oder mehr bis 0,50 mm oder weniger ausweisen und ein Abstand zwischen den benachbarten belasteten Bereichen 0,10 mm oder mehr bis 0,60 mm oder weniger beträgt, und ein Linienabstand zwischen den gepunkteten Linien in Walzrichtung 2 mm bis 10 mm beträgt.

2. Ein Verfahren zur Herstellung eines kornorientierten Elektrostahlblechs, umfassend:
Einbringen einer thermischen Spannung in ein kornorientiertes Elektrostahlblech in einer gepunkteten Linien-Anordnung, in der die belasteten Bereiche in einer die Walzrichtung des Stahlblechs kreuzenden Richtung durch Einstrahlen eines Elektronenstrahls eingefasst wurden, wobei ein Linienabstand zwischen der Elektronenstrahl-Bestrahlung in der Walzrichtung 2 mm bis 10 mm beträgt, ein bestrahlter Punkteabstand in der gepunkteten Linien-Anordnung beträgt 0,2 mm oder
mehr bis 1,0 mm oder weniger, wobei die belasteten Bereiche, die in die gepunktete Linienanordnung eingebracht werden, eine Größe von 0,10 mm oder mehr bis 0,50 mm oder weniger haben und ein Abstand zwischen den benachbarten belasteten Bereichen von 0,10 mm oder mehr bis 0,60 mm oder weniger ist, und ein Bestrahlungsenergiebetrag E pro Einheit Strahldurchmesser, die durch die folgende Formel (1) definiert ist, beträgt 30 mJ / mm oder mehr und 180 mJ / mm oder weniger, wobei: $E = \left[Beschleunigungsspannung des Elektronenstrahls \left(kV\right)\times Strahlstromwert \left(mA\right)\times Bestrahlungsdauer pro Punkt \left(μs\right)/1000\right] / Strahldurchmesser \left(mm\right)$

3. Ein Verfahren zur Herstellung eines kornorientierten Elektrostahlblechs, umfassend:
Einbringen einer thermischen Spannung in ein kornorientiertes Elektrostahlblech in einer gepunkteten Linien-Anordnung, in der die belasteten Bereiche in einer die Walzrichtung des Stahlblechs kreuzenden Richtung durch ununterbrochenes Einstrahlen eines Laserstrahls eingefasst wurden, wobei ein Linienabstand zwischen der unterunterbrochenen Laser-Bestrahlung in der Walzrichtung 2 mm bis 10 mm beträgt, ein bestrahlter Punkteabstand in der gepunkteten Linien-Anordnung beträgt 0,2 mm oder mehr bis 1,0 mm oder weniger, wobei die belasteten Bereiche, die in die gepunktete Linienanordnung eingebracht werden, eine Größe von 0,10 mm oder mehr bis 0,50 mm oder weniger haben und ein Abstand zwischen den benachbarten belasteten Bereichen von 0,10 mm oder mehr bis 0,60 mm oder weniger ist, und ein Bestrahlungsenergiebetrag E pro Einheit Strahldurchmesser, die durch die folgende Formel (2) definiert ist, beträgt 40 mJ / mm oder mehr und 200 mJ / mm oder weniger, wobei: $E = \left[durchschnittliche Laserleistung \left(W\right)\times Bestrahlungsperiode pro Punkt \left(μs\right)/1000\right] / Strahldurchmesser \left(mm\right)$

## Revendications

1. Tôle d'acier électrique à grains orientés, dans laquelle a été introduite une contrainte thermique dans un agencement en lignes pointillées où les zones à contrainte imposée ont été alignées dans une direction qui croise la direction de laminage de la tôle d'acier, où les zones à contrainte imposée introduites dans un agencement en lignes pointillées ont une taille de 0,10 mm ou plus à 0,50 mm ou moins et un intervalle entre les zones à contrainte imposée adjacentes est de 0,10 mm ou plus à 0,60 mm ou moins, et un intervalle interligne entre les lignes pointillées dans la direction de laminage est de 2 mm à 10 mm.

2. Procédé de fabrication d'une tôle d'acier électrique à grains orientés, comprenant :
l'introduction d'une contrainte thermique dans une tôle d'acier électrique à grains orientés dans un agencement en lignes pointillées où les zones à contrainte imposée ont été alignées dans une direction qui croise la direction de laminage de la tôle d'acier, par irradiation avec un faisceau d'électrons, où un intervalle interligne entre les irradiations par faisceau d'électrons dans la direction de laminage est de 2 mm à 10 mm, un intervalle entre points irradiés dans l'agencement en lignes pointillées est de 0,2 mm ou plus à 1,0 mm ou moins, les zones à contrainte imposée introduites dans l'agencement en lignes pointillées ont une taille de 0,10 mm ou plus à 0,50 mm ou moins et un intervalle entre les zones à contrainte imposée adjacentes est de 0,10 mm ou plus à 0,60 mm ou moins, et une quantité d'énergie d'irradiation E par diamètre unitaire du faisceau définie par la formule (1) suivante est de 30 mJ/mm ou plus et 180 mJ/mm ou moins, où : $E = \left[Tension d'accélération du faisceau d'électrons \left(kV\right) x Valeur du courant du faisceau \left(mA\right) X Durée d'irradiation par point \left(μs\right)/1000\right] / Diamètre du faisceau \left(mm\right)$

3. Procédé de fabrication d'une tôle d'acier électrique à grains orientés, comprenant :
l'introduction d'une contrainte thermique dans une tôle d'acier électrique à grains orientés dans un agencement en lignes pointillées où les zones à contrainte imposée ont été alignées dans une direction qui croise la direction de laminage de la tôle d'acier, par irradiation avec un faisceau laser continu, où un intervalle interligne entre les irradiations par laser continu dans la direction de laminage est de 2 mm à 10 mm, un intervalle entre points irradiés dans l'agencement en lignes pointillées est de 0,2 mm ou plus à 1,0 mm ou moins, les zones à contrainte imposée introduites dans l'agencement en lignes pointillées ont une taille de 0,10 mm ou plus à 0,50 mm ou moins et un intervalle entre les zones à contrainte imposée adjacentes est de 0,10 mm ou plus à 0,60 mm ou moins, et une quantité d'énergie d'irradiation E par diamètre unitaire du faisceau définie par la formule (2) suivante est de 40 mJ/mm ou plus et 200 mJ/mm ou moins, où : $E = \left[Puissance moyenne du laser \left(W\right) x Durée d'irradiation par point \left(μs\right)/1000\right] / Diamètre du faisceau \left(mm\right)$
